

Feb. 20, 1923.

1,446,092.

P. T. JACKSON.

REINFORCED PAPER AND METHOD OF MAKING THE SAME.

FILED OCT. 21, 1919.

2 SHEETS—SHEET 1.



Feb. 20, 1923.

1,446,092.

P. T. JACKSON.

REINFORCED PAPER AND METHOD OF MAKING THE SAME.

FILED OCT. 21, 1919.

2 SHEETS—SHEET 2.

Fig. 3.



Fig. 4



Fig. 5



Inventor:

Patrick T. Jackson  
by Robert D. Hains.

Attorney

Patented Feb. 20, 1923.

1,446,092

# UNITED STATES PATENT OFFICE.

PATRICK T. JACKSON, OF CAMBRIDGE, MASSACHUSETTS, ASSIGNOR TO PAPER PRODUCTS MACHINE COMPANY, OF BOSTON, MASSACHUSETTS, A CORPORATION OF MASSACHUSETTS.

## REINFORCED PAPER AND METHOD OF MAKING THE SAME.

Application filed October 21, 1919. Serial No. 332,201.

To all whom it may concern:

Be it known that I, PATRICK T. JACKSON, a citizen of the United States, residing at Cambridge, in the county of Middlesex and State of Massachusetts, have invented an Improvement in Reenforced Paper and Methods of Making the Same, of which the following description, in connection with the accompanying drawings, is a specification, like characters on the drawings representing like parts.

This invention relates to reenforced paper and the process or method of making the same.

It has heretofore been suggested that a reenforced paper might be formed by securing to a paper web a fleece of cotton fibres. As well understood by those skilled in the art, a fleece usually consists of short fibers which run in divers directions as the fleece comes from the card or other fleece forming machine, and that when such fleece is secured to the paper web, very little if any reinforcement is imparted to the paper strip because the fibres are short and intermingled and have no definite or predetermined direction, but on the contrary, extend in various directions, transversely, diagonally, and in other relations to the web to which the fibers are intended to be secured. Moreover, the fleece is deposited upon the paper web in a fluffy condition, and usually only the fibres next to the web become attached thereto, and even these extend in various directions relative to the paper strip. In order to impart the desired tensile strength to the paper, it is desirable to have the filaments which are connected to the paper strip, extend substantially in a longitudinal direction and be individually secured to the paper strip. The best results are secured by employing reenforcing filaments of unspun long fibres such as flax, sisal, ramie and similar long staple fibres, and adhesively securing said filaments to the paper strip while the filaments themselves are under lengthwise tension. The effect of this is that the individual reenforcing filaments or unspun long staple fibres are adhesively secured to the surface of the paper strip in substantially separated relation and extend in the substantial longitudinal direction of the paper strip, and being under tension, when thus secured to

the paper strip, they impart thereto the 55 desired reinforcement.

An important feature of the present invention comprises a paper fabric having secured thereto longitudinally of the paper fabric, a series of reinforcing filaments 60 which are adhesively secured to the paper strip while the unspun fibres are under tension.

The reinforcing filaments or unspun long staple fibres may be adhesively secured under lengthwise tension to the paper strip by some glue or adhesive, but for many purposes it is desirable that the adhesive be a waterproof material, and in carrying the invention into practical effect, such waterproof adhesive for securing the lengthwise tensioned long staple fibers to the paper, may be asphaltum or similar substance.

Another important feature of the invention comprises a process or method of forming the reenforced paper, which consists in adhesively securing the separate reinforcing filaments to the paper web while the filaments are under lengthwise tension.

The method may be carried into effect 80 by various means, one good form of which is illustrated in the accompanying drawings.

In the drawings:—

Fig. 1 is a perspective view of a machine 85 for separating and laying long staple fibres in parallel longitudinal relation and maintaining them under lengthwise tension as they are applied to a paper web;

Fig. 2 is a sectional detail showing the 90 fibres being applied between two plies of paper web;

Fig. 3 is a face or plan view showing a paper web having adhesively secured thereto long staple unspun fibres or filaments 95 which are held in lengthwise tension and straightened condition by the adhesive;

Fig. 4 is a plan or face view showing on an enlarged scale, a narrow section as it is divided from the web of Fig. 3; and

Fig. 5 is a perspective view showing one of the uses to which the reenforced paper may be applied as for instance, in the form of a twisted thread.

The character of the reinforcing filaments 105 which may be applied under lengthwise tension to the paper web or strip, may be of suitable character, but more particularly

the present invention has in view the application of long staple unspun fibres, such as flax, sisal and the like, and in illustrating a machine for carrying the invention into practical effect, a mechanism adapted to operate on such long staple unspun fibres is shown.

In the drawings, and more particularly referring to Fig. 1, the long staple fibre *a* 10 consists of sisal or flax fibre, which after it has been scutched and has had the woody matter removed therefrom, is fed between the feed rolls 1 and 2 for delivering the fibre to a hackling or drawing-out and tensioning process. In the present instance of the invention, the feed rolls 1 and 2 are driven from a suitable source of power as by means of the belt 3 which passes over a driving pulley 4 connected to one of the 20 feed rolls. A spring 5 may be advantageously employed and adjusted by a hand wheel 6 for maintaining the feed rolls 1 and 2 in proper working relation.

The long staple fibres *a* after passing between the feed rolls 1 and 2 are fed lengthwise to the drawing or tensioning means either direct or by means such as an apron or belt 7 which passes over the end rolls 8 and 9 and under the roll 10, the construction being such that as the long staple fibres *a* are delivered by the feed rolls, they are carried to the drawing-out and tensioning mechanism, as will presently appear.

The roll 9 may be driven from a suitable 35 source of power, in the present instance, a pulley 10 as indicated is driven by a belt 11 which also extends over a pulley 12 connected to the shaft 13 of the roll 14. Above the roll 9 is another roll 15 which serves 40 to maintain the elongated fibres in contact with the apron 7 at the pinch between the rolls 9 and 15, and as such elongated fibres pass to the drawing or tensioning means.

Suitably mounted on the machine frame 45 in co-operative relation with the roll 14 is another similar roll 16 over which roll passes the hackling or drawing and tensioning apron. In the present instance of the invention, the drawing or hackling apron 50 as it may be called, comprises a series of slats or rods 17, which are connected at their ends to sprocket chains 18 which pass over sprocket wheels carried by the rolls 14 and 16 respectively. Each of the slats or rods 55 17 is provided with a series of pins which extend upwardly therefrom as indicated at 19, and as the pins rise from the under portion of the roll 14, these pins enter between the elongated fibres *a* as they emerge between the rolls 9 and 15. The drawing or 60 hackling apron 17 may have a greater surface speed than the speed of delivery of the elongated fibres *a* from between the rolls 9 and 15, the effect being that the fibres *a* 65 are not only drawn into parallel relation by

the pins, but they are placed under lengthwise tension, and while under this tension, the fibres, now appearing in substantially parallel relation as at *b*, pass into the bight between the delivery rolls 20 and 21. The 70 rolls 20 and 21 are preferably given a somewhat faster surface speed than the speed of the elongated and tension fibres at *b*, the effect being that an additional lengthwise tension is given to the fibres at *b*, which serves to 75 further insure substantial parallelism between the fibres and hold them under lengthwise tension. The rolls 20 and 21 may be suitably driven, but in the present instance, the roll 20 is provided with a driving pulley 22 which is driven by a belt 23 actuated by a suitable source of power, and a spring 24 which may be similar to the spring 5 serves to hold the rolls 20 and 21 in operative relation, the construction being such 85 that as the long staple fibres *b* emerge from the bight of the rolls 20 and 21, they are in substantial parallelism and under tension, and while in such condition, the present invention contemplates that the filaments or 90 long staple fibers may be adhesively attached to the paper web.

In the present instance, the paper web is indicated at *c*, and travels in the direction of the arrow from a suitable supply 95 over a guide roll 25, and then under a roll 26 where it is supplied with an adhesive from a roll 27. The roll 27 may be supplied with the adhesive in any suitable manner, but as indicated in the present instance, 100 it rotates partially submerged in the adhesive 28 contained in a tank or receptacle 29. The adhesive is preferably water-proof so that when applied to the paper as indicated by the dots at *d* (Fig. 1), the waterproof adhesive imparts a waterproof character to the paper web.

The paper web passes from between the adhesive roll 27 and the roll 26 over the guide roll 30 which is so positioned relative to the roll 20 that as the straightened and tensioned long staple fibres emerge from between the rolls 20 and 21 they are forced into intimate contact with the adhesive surface of the paper web or fabric between 115 the rolls 20 and 30. The roll 20 may be heated by any suitable heat medium which in the present instance may be circulated through the roll 20 by a pipe, the conditions being such that the roll 20 will be sufficiently heated to prevent objectionable accumulation of the adhesive thereon and permit the tensioned and straightened fibres being pressed onto and adhesively engage the sticky surface of the paper. It is desired a 120 cooling blast of air may be projected upon the surface of the web by means of a pipe 31 connected by a conduit 32 with a suitable supply, but this is not always necessary.

The paper web *c* passes from the roll 30 130

over a supporting and feeding roll 33 which may be driven by a suitable belt 34 and pulley 35, deriving their motion from a suitable source of power. In order that 5 the feeding roll 33 may impart to the paper web a travel somewhat in excess to the speed of the reinforcing filaments *b* to thereby cause the filaments to be maintained under lengthwise tension as they are adhesively 10 secured to the paper web, the paper web may be supplied with the adhesive throughout its surface, except at the marginal portions 36 on which bear the idle rolls 37 which co-operate with the feed roll 33 to 15 give to the paper web its desired movement.

From the construction described it will be clear that the filaments, which may preferably be unspun fibres of long staple, are 20 first arranged in substantial parallel relation, and then while in such parallel relation and under lengthwise tension, they are adhesively secured to the surface of the paper web, so that they impart to the paper 25 a substantial and definite reinforcement and are in substantial parallel relation.

It will sometimes be desirable to enclose the longitudinal reinforcing filaments between two plies of paper, and a construction 30 which may be employed for this purpose is indicated by Fig. 2, wherein the frame of the machine 38 supports the standard 39 at a point in advance of the drawing and hacking apron, and on the standard 39 are 35 the drawing and guide rolls 40 and 41 between which pass the paper webs 42 and 43 as indicated by the arrows. The longitudinally extending and lengthwise tension fibres at *b* (Fig. 2) pass between the two 40 plies of paper 42 and 43 as indicated in Fig. 2, and then the duplex fabric is drawn longitudinally by the drawing or feed rolls 44 and 45, the construction being such that by operating the rolls 40, 41, and 45 44, 45 at somewhat increased speed relative to the speed of the fibres, the filaments or fibres of long staple *b* are secured to the paper webs in parallel relation and under lengthwise tension. When the fibres or 50 filaments have been secured to the paper web, it may be dried and thus provide a strong and durable wrapping material for general use, or, if desired, it may be subsequently treated to form threads, as will 55 now be described.

In Fig. 3 the elongated and lengthwise tension filaments *b* are shown as extending in substantial parallel relation longitudinally of the paper web to which they 60 have been adhesively secured, preferably by waterproof material, as hereinbefore described. When properly dried and ready for further treatment, the paper web may be divided into strips *f* along the lines 65 *x*—*x* as indicated in Fig. 3, thereby pro-

ducing a paper strip *f* reenforced by longitudinally extending fibres *b* under lengthwise tension. The strips *f* and the attached fibres may then be twisted into a thread *g* as indicated in Fig. 5, the length of the 70 fibres being such that they extend with the paper a plural number of times about the axis of the thread thus formed.

The paper strip and longitudinally extending fibres may be twisted so as to present the paper surface outwardly throughout the length of the thread, or it may be twisted to present the water-proof and fibrous surface outwardly. The threads thus formed may be advantageously employed 75 for a great variety of purposes. The essentials of the present invention consist in the method of making the reenforced paper and also in the reenforced paper itself, which preferably may consist of more than one 80 layer having longitudinally extending reinforcing unspun fibres of long staple secured adhesively to the paper strip or paper strips under longitudinal tension.

The reenforced paper fabric described is 85 adapted for a great variety of uses, such for instance, as wrappers, covers for shipment of substances of various kinds, cases, and in fact, as a general substitute for the more expensive materials now generally used. The 90 terms "paper fabric," "strip," and "web" are used in their general sense and where more than one paper fabric strip or web is used to form the composite fabric, the reinforcing filaments may be enclosed advantageously between two of them, and such 95 paper fabrics, strips, or webs, may be of the same or of different thicknesses.

What is claimed is:—

1. The method or process of forming reenforced paper, which consists in adhesively securing a series of unspun fibres to a paper web in longitudinal relation under lengthwise tension.

2. As an article of manufacture, reenforced paper, comprising in its construction, a paper fabric which has a waterproof adhesive applied to one face thereof, a series of unspun fibres which extend in substantially parallel relation longitudinally along the surface of the paper fabric and are secured thereto under lengthwise tension by the waterproof adhesive.

3. As an article of manufacture, reenforced paper, comprising in its construction, a paper fabric which has a series of separate unspun fibres of long staple extending longitudinally thereof and adhesively secured thereto under lengthwise tension.

4. As an article of manufacture, reenforced paper, comprising in its construction, a paper strip which has asphaltum applied to one surface thereof, a series of long unspun fibres which extend in substantially parallel relation longitudinally of the paper

- 4
- strip and are secured thereto by the asphaltum under longitudinal tension, and a second strip of paper superposed on the first strip and adhesively secured thereto.
5. The method of making reenforced paper, which consists in feeding a sheet of unspun fibres lengthwise, exerting a longitudinal pull upon the fibres as they are fed lengthwise, feeding a sheet or web of paper lengthwise, applying an adhesive to the surface of the sheet or web as it is fed lengthwise, and applying the unspun fibres to the adhesive on the paper sheet or web while the unspun fibres are under lengthwise tension.
10. The method of forming reenforced paper having a series of unspun fibres of long staple adhesively applied thereto in substantially parallel relation and under lengthwise tension, which consists in adhesively securing leading portions of unspun fibres to a traveling paper sheet, exerting a retarding force upon the trailing portions of the fibres to place lengthwise tension on the fibres as the fibres are applied to the paper sheet, and finally freeing the trailing portions of the unspun fibres as they move with the paper sheet.
15. The method of forming reenforced paper having a series of unspun fibres of long staple adhesively applied thereto in substantially parallel relation and under lengthwise tension, which consists in adhesively securing the leading portions of unspun fibres to a traveling paper sheet, and exerting a retarding force on the trailing portions of the fibres to tension the fibres lengthwise as they are drawn longitudinally by the traveling paper sheet.
20. The method of forming reenforced paper having a series of unspun fibres of long staple adhesively applied thereto in substantially parallel relation and under lengthwise tension, which consists in adhesively securing leading portions of unspun fibres to a paper sheet and exerting a longitudinal pull upon the fibres as they are applied to the paper sheet.
25. The method of forming reenforced paper having a series of unspun fibres of long staple adhesively applied thereto in substantially parallel relation and under lengthwise tension, which consists in feeding a mass of unspun fibres from a source of supply, advancing a paper sheet longitudinally at a speed greater than the speed of the unspun fibres, applying the leading portions of the unspun fibres adhesively to the faster traveling paper sheet to draw out the fibres and place them under lengthwise tension on the adhesive surface of the paper sheet.
30. As an article of manufacture, reenforced paper comprising in its construction, a paper strip which has a series of separate unspun fibres of long staple adhesively applied thereto under lengthwise tension in a single layer of substantially the same thickness as one of the fibres, and with the fibres lying in substantially parallel relation.
35. The method or process of forming a reenforced paper, which consists in adhesively securing a series of substantially parallel non-continuous unspun fibres of comparatively long staple to a paper web in longitudinal relation under lengthwise tension.
- In testimony whereof, I have signed my name to this specification.

PATRICK T. JACKSON.